

Patented Oct. 4, 1927.

1,644,425

# UNITED STATES PATENT OFFICE.

CHARLES A. GEATTY, OF ELKRIDGE, MARYLAND.

## ALLOY.

No Drawing.

Application filed April 14, 1925. Serial No. 23,088.

This invention relates to alloys and especially to an alloy for brake bands, transmission bands and the like.

Brake bands and transmission bands as commonly used on automobiles and other machinery consists generally of a flexible steel band encircling or fitting within a drum on a revolving part and provided with a lining to bear against the drum. The linings most frequently used for this purpose are some form of fabric frequently containing a wire mesh foundation, although leather and wood are also used for such linings. Such linings are open to the objections that they quickly become burnt or glazed under conditions of use, are hygroscopic and expand and contract with the changes in atmospheric conditions, and tend to slip when wet or oily. Furthermore, continuous application of such brakes results in heating the drum and causing the brakes to grip.

Metal linings have been proposed for the purpose but those hitherto used have been found deficient in braking effect or subject to the same objections as the fabric linings.

I have found, however, that a properly proportioned alloy may be made which will be free from the objections inherent to the fabric, leather or wood linings and which will have ample braking effect when in use.

One important object of the present invention, therefore, lies in the production of an improved alloy especially adapted for use in connection with brakes, transmission bands and the like as a lining or work-engaging surface therefor.

A second important object of the invention is the production of an improved alloy for these purposes which may be rolled to form with great ease, is capable of being machined without difficulty, has a proper rigidity to prevent its buckling when riveted to the band, and does not readily wear under conditions of use.

It is also to be noted that, due to the long life of the lining thus made much of the constant adjustment needed with the usual type of brake linings is eliminated and greater safety in the operation of automobiles and the like is assured.

For this purpose I have found that the alloy should contain certain metals having no chemical affinity and that an alloy of lead, antimony and copper to which has been added a certain proportion of sulphur makes an excellent material for the purpose. I have also found that the lead should be largely in excess of the other constituents and that an alloy, containing by weight 95% of lead 3% of antimony and 2% of copper, to which is added 5% by weight of sulphur is most suitable for use as a lining for brake bands although these proportions may be varied somewhat in accordance with the particular use for which the lining is intended.

To make this alloy I preferably fuse together 95 pounds of lead, 3 pounds of antimony and 2 pounds of copper and then add to the fused and thoroughly mixed mass 5 pounds of sulphur. The mass thus formed may then be cast into ingots and rolled or extruded to the desired cross section.

The alloy thus made is formed to meet all the requirements for use as a lining for brake bands, transmissions and the like.

Having thus described the invention, what is claimed as new, is:

1. An alloy for linings for brake bands and the like containing by weight lead 95%, antimony 3% and copper 2%.

2. An alloy for linings for brake bands and the like and containing lead, antimony, copper and sulphur in the proportions of 95 pounds of lead, three pounds of antimony, two pounds of copper and 5 pounds of sulphur.

3. An alloy for linings for brake bands and the like containing lead, antimony, copper and sulphur, the lead constituting at least nine-tenths of the entire alloy by weight, the weight of the sulphur being substantially that of the antimony and copper and the weight of the antimony being slightly in excess of the weight of the copper.

In testimony whereof I affix my signature.

CHARLES A. GEATTY.